

## UNITED STATES PATENT OFFICE

2,569,894

ALLOYED STEEL SUITABLE PREFERABLY  
FOR WATER HARDENING TOOLS OF HIGH  
RESISTANCE TO WEAR AS WELL AS SHOCKHelmuth Krainer and Karl Swoboda, Kapfenberg,  
Austria, assignors to Gebr. Böhler & Co.  
Aktiengesellschaft, Vienna, AustriaNo Drawing. Application February 27, 1948, Se-  
rial No. 11,874. In Germany October 31, 1941Section 1, Public Law 690, August 8, 1946  
Patent expires October 31, 1961

3 Claims. (Cl. 75--123)

1

The invention relates to an alloy steel suitable preferably for water hardening tools of high resistance to wear as well as shock.

For such tools, especially for turning tools, for grooving or rifling tools and drawing dies, alloyed steels are used having a hardness of RC of at least 67, preferably 68 to 69 in the hardened state. The hardness should not decrease appreciably when tempered at a temperature of approx. 200° C., at least the hardness should not drop to less than 66 RC.

It is, however, not possible to choose a suitable alloyed steel merely according to the hardness obtainable. As the tools under consideration are used for extremely hard works, and as they are subjected to mechanical wear, they have to contain in their micro-structure carbides of very great hardness embedded in a hard matrix. As is commonly known, steel of high carbon content is chosen and this steel is alloyed with the carbide forming elements chromium, vanadium and tungsten, tungsten representing the main addition, the known alloys having a content of mostly more than 1% C, up to 1.5% Cr, up to 0.5% V and 4 to 8% W. The content of tungsten may be reduced to 2%. The high content of tungsten causes brittleness of the tool.

According to the present invention the content of tungsten is decreased below the hitherto known minimum by a variation in the relative amounts of the carbide forming elements. According to the invention alloyed steels are to be used containing, besides iron and the usual impurities, the components enumerated below:

1.0 to 2.0% carbon  
0.8 to 2.5% vanadium  
0.5 to less than 2% tungsten

The steels may also have a content of chromium of less than 1%.

The alloy to be used according to the present invention is found to display its extremely favourable properties most reliably if the concentrations of the carbide forming elements are kept within relatively close limits. Especially suitable is the alloy containing besides iron and the usual impurities

1.3 to 1.8% carbon  
0.1 to 0.6% chromium  
1.6 to 1.75% vanadium  
1.0 to less than 2% tungsten

In tests the best results were obtained with a steel of the following composition:

1.6% carbon  
0.3% chromium  
1.4% vanadium  
1.6% tungsten

2

balance iron and the usual impurities. After quenching this steel in water from a temperature of 780-840° C. a RC hardness of 65-70 is obtained.

No decrease in hardness occurs on tempering at 100° C. Tempering at 200° C. does not decrease the RC hardness below 66.

Steel to be used according to the present invention proved in tests not only equal to a steel normally used for rifling tools with a tungsten content of 8% but was even superior in many cases.

The main advantage of the alloy used according to the present invention as compared with the steels normally known to be used for rifling tools and having a high content of tungsten is its greater toughness. Accordingly its application is not only valuable for rifling and grooving tools or drawing dies but generally for tools exposed to excessive wear and shock.

20 What we claim is:

1. Water hardening alloy tool steel having an RC hardness in the range of 65 to 70 and containing

1.0 to 2.0% carbon  
0.8 to 2.5% vanadium  
0.5 to less than 2% tungsten

balance iron and impurities.

2. Water hardening alloy tool steel as defined in claim 1 containing additionally a small quantity, less than 1% of chromium.

3. Water hardening alloy tool steel having an RC hardness in the range of 65 to 70 and containing

1.3 to 1.8% carbon  
0.1 to 0.6% chromium  
1.0 to 1.75% vanadium  
1.0 to less than 2% tungsten

balance iron and impurities.

40

HELMUTH KRAINER.  
KARL SWOBODA.

## REFERENCES CITED

45 The following references are of record in the file of this patent:

## UNITED STATES PATENTS

Number Name Date  
1,496,980 Armstrong ----- June 10, 1924

## FOREIGN PATENTS

Number Country Date  
180,112 Switzerland ----- Dec. 16, 1935

55